

Nov. 16, 1926.

1,607,220

B. P. VON EHRENTHAL ET AL

PROCESS AND DEVICE FOR PRODUCING COTTONIZED FIBERS

Filed Feb. 26, 1924

5 Sheets-Sheet 1

Fig. 1.



Fig. 2a.

Fig. 2.



Fig. 3.



Fig. 4.



Inventors  
B. P. von Ehrenthal  
C. Scholz  
By Markos Clark  
*Attest.*

Nov. 16, 1926.

1,607,220

B. P. VON EHRENTHAL ET AL

PROCESS AND DEVICE FOR PRODUCING COTTONIZED FIBERS

Filed Feb. 26, 1924

5 Sheets-Sheet 2



Inventors  
B. P. von Ehrenthal  
C. Scholz  
by Markman Clerk  
Hibbs

Nov. 16, 1926.

1,607,220

B. P. VON EHRENTHAL ET AL

PROCESS AND DEVICE FOR PRODUCING COTTONIZED FIBERS

Filed Feb. 26, 1924

5 Sheets-Sheet 3



Inventors  
B. P. von Ehrenthal  
C. Schopff  
By Marks & Clark  
1924

Nov. 16, 1926.

1,607,220

B. P. VON EHRENTHAL ET AL

PROCESS AND DEVICE FOR PRODUCING COTTONIZED FIBERS

Filed Feb. 26, 1924

5 Sheets-Sheet 4

Fig. 11.



Fig. 12.



Inventors  
B. P. von Ehrenthal  
C. Sczpolz  
by Marks & Clark  
Attys.

Nov. 16, 1926.

1,607,220

B. P. VON EHRENTHAL ET AL

PROCESS AND DEVICE FOR PRODUCING COTTONIZED FIBERS

Filed Feb. 26, 1924

5 Sheets-Sheet 5

Fig. 15.



Fig. 13.



Fig. 14.



Inventors  
B. P. von Ehrenthal  
C. Strobl  
by Marks & Clark  
1926.

Patented Nov. 16, 1926.

1,607,220

# UNITED STATES PATENT OFFICE.

BRUNO POSSANNER VON EHRENTHAL, OF COTHEN-ANHALT, GERMANY, AND KARL SCHOLZ, OF TETSCHEN, CZECHOSLOVAKIA.

## PROCESS AND DEVICE FOR PRODUCING COTTONIZED FIBERS.

Application filed February 26, 1924, Serial No. 695,385, and in Germany March 28, 1923.

This invention relates to processes and devices for producing cottonized fibers.

In cottonizing bast fibers (half-clean hemp, flax, nettle and the like) it has been found that the extraction of the fiber can be accomplished to any desired extent by the most diverse chemical opening, washing, and loosening processes applied to wet or dry material, but that the cottonized product obtained by all these processes is very different in quality, etc., so that parts of it contain bundles of cells, and individual cells weakened by chemical action and destroyed by mechanical treatment, so that a very non-uniform staple is obtained and the fibers are partly hard and brittle, and partly fragile due to chemical action, and consequently give little satisfaction in the subsequent spinning process, so that instead of fine uniform threads coarse uneven threads only can be obtained as in spinning waste, and also frequent breakages of fleeces and threads, considerable waste, and a low efficiency of the spinning machines occur.

Years of experience in testing plants have shown that by these methods alone a real high grade substitute for cotton cannot be obtained by cottonizing but that, apart from the preliminary treatment of the fibrous substance, a particular mechanical treatment, which damages the fibers as little as possible, is necessary, in order to accomplish the requisite uniform solution into individual cells without injuring and shortening the natural cell and to obtain in this manner a very soft, woolly and clean fiber product of great strength which can be regarded in the spinning mill as a complete equivalent of cotton. The object of this invention is to provide processes and devices for obtaining these results.

The raw fibrous substance, or a substance which has been deshived or subjected to any preliminary chemical or mechanical treatment, is dealt with as follows:

1. It is squeezed or beaten and simultaneously treated with warm or cold water or liquid chemicals.
2. It is gradually but rigorously stretched when wet in a cold or warm condition, whereby the individual cells are extracted from the cell conglomeration but without completely breaking the strands or the fleece.
3. The fibrous substance is separated in a cold or warm condition into individual cells

by jets of water or liquid directed against one or both sides of the fibrous substance or fleece, this liquid serving to separate and wash out the loosened individual cells from the conglomeration and to completely dissolve and remove the incrustations and adhesive substances.

The fibrous substance, which has been treated in this manner and dissolved into individual cells, i. e. cottonized, can be either immediately deprived of liquid and dried, or it may be bleached, impregnated, roughened, dyed and subjected to the usual processes in the flock before it is deprived of liquid and dried.

The cottonized fibrous material produced in this manner is not only completely clean and dissolved into uninjured individual cells but, in consequence of the described treatment, will be found to surpass fibrous substances cottonized in any other way as far as softness, spinning qualities and particularly tensile strength is concerned. Since, if the machines and apparatus are arranged in a suitable manner, no manual labor beyond the feeding of material into the first machine is required, the economy of the process is completely secured, particularly as the output and quality of the product is improved.

Although the aforesaid three processes can be carried out with various machines and apparatus, certain arrangements and types have been found to be particularly advantageous and these form further features of the invention. These machines and devices are illustrated in the drawing in which—

Figs. 1 and 2 are a section and a front elevation of a drawing device consisting of pairs of rolls,

Fig. 2<sup>a</sup> shows a cross section of a modification of Fig. 1 in which the rollers are partly submerged in a suitable liquid.

Figs. 3 and 4 illustrate the action of the drawing rollers on the cells of a bundle of fibers.

Figs. 5, 6 and 7 show a modified drawing device, Figs. 5 and 6 being fragmentary sections with the parts shown at different moments of operation and Fig. 7 being a fragmentary elevation partly in section.

Figs. 8-12 illustrate three different forms of a device for squirting liquid against the fibrous substances, Fig. 8 being a side eleva-

60

65

70

75

80

85

90

95

105

110

tion partly in section, Fig. 9 a cross section and Fig. 10 a fragmentary cross section on an enlarged scale of one form of squirting device, Fig. 11 a section of a squirting device provided with perforated bands and Fig. 12 a section of a squirting device in which the fibrous substance passes through a pair of rollers and then receives liquid from nozzles or openings arranged at opposite sides of the fibrous substance issuing from the pair of rolls.

Figs. 13-15 show a bruising or beating machine, Fig. 13 being an end view, Fig. 14 a partial front elevation and Fig. 15 a detail.

In accordance with the invention the fiber containing plant stalks after being deshived are first subjected to a preliminary opening treatment in beating, crushing or bruising devices which may be constructed as shown in Figs. 13-15, which devices are more fully described hereinafter. After this preliminary treatment the material is then stretched in a moist condition in a stretching device. This stretching device may be of any preferred kind as shown in Figs. 1-7. By this stretching operation the individual cells or fiber elements are separated from each other or loosened in their cell conglomeration. The fibrous material in the form of a moist fleece  $z$ , is fed into a pair of rollers  $a, b$ , Fig. 1 in which the ends of the individual cells  $j$  adhering to each other as indicated diagrammatically in Fig. 3 are gripped. The drawing device in Fig. 1 or 2<sup>a</sup> has a pair of rollers  $a, b$  which revolve in the direction of the arrows and another pair of rollers  $c, d$  which revolve similarly as the rollers  $a, b$  but at a somewhat higher speed. The surfaces of the rollers may be provided with small grooves, roughened or coated with a suitable covering. The rolls are journaled in a usual manner in bearings  $e, f$  and are coupled to each other by toothed wheels  $g, g$  so that the rolls of each pair are revolved uniformly. Each pair of rolls seizes the fleece  $z$  in a straight-line bite. The distance between the bites of the pairs of rolls corresponds to the average natural length of the cells of the cottonized fibers. On account of the slightly greater speed of the front pair of rollers  $c, d$  a gentle pull is exerted on the cells of the fleece. Each length of fleece corresponding to the distance  $x-y$  is stretched in accordance with the difference of speeds to a distance  $x'-y'$  as indicated in Fig. 4. Since the distance between the bites corresponds to the length of the cells tearing of the individual cells is avoided and they are drawn apart or separated from each other as indicated in Fig. 4. The separation of conglomerations or groups of cells into individual cells can then be easily carried out. Instead of having only two pairs of rolls several pairs may be

arranged one behind the other in a suitable manner.

In Fig. 2<sup>a</sup> the conveyers 400 and 401 are shown that carry the fibers into and away from the rollers which are partly submerged in a liquid such as diluted sodium hydroxide solution in a trough 402.

Instead of the continuously acting drawing rollers of Figs. 1 and 2 other forms of drawing devices, in which the retarding rolls  $a, b$  are substituted by other clamping devices such as clamping bars or the like, may be employed. A device of this kind is shown in Figs. 5-7 in which the fleece  $z$  is stretched by flat clamping members. In this device there is a roller which may be moved step-by-step by a ratchet and pawl device, and is provided at its periphery with movable bars  $t$ . The roller or drum  $w$  is provided with radial guide pins  $h$  which coact with two ends of each of the bars  $t$ . Arranged at the ends of the drum  $w$  are stationary rings  $s$  with vertical faces  $u$  and  $a$  overhanging rim  $j$  which limit the outward travel of the bar  $t$ . Springs, such as leaf springs  $v$ , in the rings tend to press the bars  $t$  outwardly. The ring  $s$  is formed with a guide ring  $m$  that extends into notches or slots in the ends of the bars  $t$ .

This guide ring  $m$  has a gap at the top of the drum  $w$  see Fig. 7 through which each bar  $t$  can be pushed down onto the drum, as shown in Fig. 5, as it arrives at the top of the drum  $w$ . At this point, opposite to the bar  $t$  at the top of the roller, there is a reciprocating pressure member  $r$  which is moved up and down periodically by an eccentric or cam rod  $o$ . During its reciprocating motion the pressure member is guided in a vertical guide way  $p$ . Arranged above the pressure member  $r$  is a loading or holding device  $q$  with clamping surfaces  $n$ . The stretching of the fiber is accomplished by turning the drum  $w$  with the fibrous material upon it through an angle corresponding to the width of one bar  $t$  without pressing the fleece against the roll  $w$  by the pressure member  $n$ . Immediately after each turn of the drum  $w$  through the said angle, the pressure member  $r$  together with the clamping member  $q$  is lowered, so that the clamping surfaces  $n$  engage with the fibers as indicated in Fig. 5 so as to hold them firmly at the clamping points, the pressure against the member  $q$  being exerted by a spring  $i$  whose tension can be regulated. The pressure member  $r$  continues its downward travel after the clamping action of the clamping surfaces  $n$  has taken place, so that the bar  $t$  is depressed and the fibers are bulged downwards and a stretching action as indicated in Fig. 5 is accomplished. The pressure member  $r$  thereupon rises in the gap in the ring  $m$  and returns to its normal position and the clamping action of the sur-

faces *n* ceases. The drum is then rotated another step and a fresh downstroke of the pressure member *r* takes place to push down the next bar *t* into gap in the ring *m*. The distance between the bites or clamping surfaces *n* is such that the individual cells are drawn apart as in the case of the device illustrated in Figs. 3 and 4 without the cells being torn to any appreciable extent.

10 After the fibers having stretched or drawn apart they are treated with liquid squirted against them by a suitable device which forms another feature of the invention.

Three forms of a suitable squirting device 15 are shown in Figs. 8-12, which are adapted to separate the individual cells through the action of jets of liquid under pressure without tearing the bundles of fibers. In accordance with the invention the fibrous substance 20 which has been subjected to a preliminary treatment is fed continuously in the form of a thin fleece in a device of the kind illustrated in which it is held at a certain point by the application of pressure and subjected at a certain distance from this point to the action of liquid jets under pressure directed toward the fleece from both sides at an oblique angle. The jets exert a vigorous pull on the fleece by which the 25 loosened individual cells are pulled and washed out. The distance between the point at which the fibers are held and the point of impact of the jets is variable and must be adapted to the fibrous substance under treatment, that is to say to the natural length of the cells. In flax or hemp fibers the average natural length is about 40 mms., so that in handling fibrous material of this kind this 30 distance will have to be chosen so that the individual cells, and these only, are separated and washed out of the crushed and stretched fibrous material by the liquid jets. The individual cells or fiber elements thus 35 washed out are caught up by suitable means, such as a sieve.

Referring to Figs. 8-12 of the drawing 100 is a fleece consisting of fibrous material which has been subjected to a preliminary treatment. The fleece is fed into the bite between two rollers 105, which have exterior surfaces of suitable form so as to seize the fleece 100 and move it forward at a uniform speed. The rolls are journaled in bearings 107, 110 and are coupled to each other by toothed wheels 111 whose size is such as to cause the rolls to revolve at identical peripheral speeds in opposite directions. The rolls hold the fleece firmly in their bite without shifting the fibers relatively to each 50 other.

Each roll 105 has a core formed with radial chambers 101 distributed around the periphery of the roll and closed by an external shell or cylinder 102. The cylinder 55 102 has oblique channels or perforations

which lead from its chamber 101 in the direction of movement of the fibrous material (see Fig. 10). At one or both ends of each roll there is arranged a head 108 provided with connection pipes 106 adapted to be connected to water supply pipes. A ring 112, which revolves with the roll and is slotted opposite to each chamber 101, and a disk 113 firmly fixed to the head 108 form a watertight joint between the interior of the roll and its head. Each disk 113 has an opening 104 which is connected through a channel 114 with the interior of the respective head 108. If necessary the heads 108 can be turned a short distance around the shafts of the rolls so that the position of the opening 104 in the disk 113 can be correspondingly altered, see Fig. 10.

When the squirting device is in operation the fleece 100 seized by the rolls 105 is progressively held at its various points in the bite between the rollers. Water under pressure enters through the opening 104 into one or more chambers 101 which lie at the side of the bite where the fleece is discharged from the rollers. The jets act upon the cells in the bite between the rolls and tend to clamp the fibers more firmly together and yet to separate them into their elements. As the rollers revolve the jets also exert a gentle stretching effect by seizing individual cells and tending to move them in the direction in which the fibers are moved. Since the seizure of the fibers by the jets takes place whilst the cells are still held in the bite between the rolls, a separation of entire bundles of fibers is prevented. By turning the heads, and thus shifting the opening 104, the path in which the squirting action is effective can be adjusted within the required limits and the angle at which the jets impinge upon the fleece can thus also be varied.

In the modification shown in Fig. 11 the fleece 205 is fed forward between two coarse meshed shifting cloths 204 which pass over rolls 202. At one point two pressure bars 203 or the like held in elastic supports press the fleece 205 together so that it is firmly held at this point. When the fleece has passed beyond the said bite it is subjected to the action of oblique water jets that issue from oblique passages in the walls of squirting members 201. The action of the oblique jets is similar to the effect of the jets of the device shown in Figs. 8-10, for in this device also jets act directly on the cells which are still held in the bite and a loosening of entire bundles of fibers is thus avoided. The position of the squirting members 201 with respect to the bite is adjustable.

In the arrangement shown in Fig. 12 the fleece is clamped between two solid rolls whose external surfaces may, if necessary, be specially adapted to exert a vigorous seizing effect by being grooved, roughened,

etc. The squirting, washing and stretching of the fibers is effected with jets of water under pressure issuing from oblique passages 208 in the walls of hollow squiring members 210 similar to the members 201 of Fig. 11. The squiring members 201 may be provided at the edges near the rollers 207 with sharp edges 209 which act as scrapers.

The fiber elements or cells finally extracted from the fibrous substance by the liquid jets as described are subsequently dried in any suitable manner. The liquid may be removed from these fibers by squeezing them or by placing them in a drum or the like which is rotated at a suitable speed to expel the liquid by centrifugal force. The drying process may also consist in conveying the separated cells or fiber elements on bands through hot air. The particular form of device per se used for removing the liquid and thoroughly drying the extracted cells or fiber elements may be of any desired type.

The extracted fibers are of course bleached when desired in any known manner as by means of solutions of active chlorine. The fiber elements may also be sized or impregnated with fatty substances, such as oil, soap or the like.

The bruising or squeezing operation in accordance with the invention may be carried out by a device or machine as shown in Figs. 13-15. The fibrous substance is placed on a conveyer belt 300 which may consist of an endless metal web and passes over rolls 301, and the belt feeds the fibrous substance in a wet condition while warm or cold into a beating device consisting of wooden rams 302 adapted to be raised and lowered by cams 304 so as to strike against blocks or tables 306 beneath the metal web, the striking effect of the rams being enhanced and made elastic by springs 305 which have the additional effect of throwing the ram upward immediately after each stroke. By staggering the cams the rams can be caused to perform their strokes in succession in any desired order and by adjusting the lengths of the cam rods the drop of each ram may be varied. Any number of rams may be used and the operation of any individual ram or rams may be stopped at will. Arranged between the rams are water outlets 310 through which cold or warm water or any suitable liquid chemical may be caused to pour onto the fibrous material on the belt. The belt or cloth conveyer carries the fibrous material into the gaps between the rams 302 and their blocks and the blows administered by the rams squeeze out the washing liquid which flows away through the metal web while the fibrous material, after passing from beneath the ram, absorbs fresh liquid from the other pipes. By this alternate wetting and squeezing out of the moisture by the strokes of the ram an excellent mechani-

cal washing effect is accomplished and, on the other hand, by the strokes administered by the ram, together with the swelling of the material by the liquid from the pipes, a better and more uniform distribution of the fibrous material over the conveyer belt is gradually achieved. This may be extremely important for the feeding of material into other machines in which the material might subsequently be treated.

We claim:

1. Process for producing cottonized fibers consisting in treating the fibrous substance so as to soften the fiber, stretching the substance, separating the elements of the fibers by directing liquid jets against it, and then depriving it of liquid and drying it.

2. Process for producing cottonized fibers consisting in treating the fibrous substance so as to soften the fiber, squeezing and stretching the substance, separating the elements of the fibers by directing liquid jets against it, and then depriving it of liquid and drying it.

3. Process for producing cottonized fibers consisting in treating the fibrous substance so as to soften the fiber, beating and stretching the substance, separating the elements of the fibers by directing liquid jets against it, and then depriving it of liquid and drying it.

4. Process for producing cottonized fibers consisting in treating the fibrous substance so as to soften the fiber, stretching the substance, separating the elements of the fibers by directing liquid jets against it, bleaching, and then depriving it of liquid and drying it.

5. Process for producing cottonized fibers consisting in treating the fibrous substance so as to soften the fiber, stretching the substance, separating the elements of the fibers by directing liquid jets against it, bleaching, and sizing, and then depriving it of liquid and drying it.

6. Process for producing cottonized fibers consisting in treating the fibrous substance so as to soften the fiber, stretching the substance, separating the elements of the fibers by directing liquid jets against it, bleaching, sizing and dyeing, and then depriving it of liquid and drying it.

7. A process for producing cottonized fibers consisting in beating the fibrous substance by a number of beating devices, wetting the fibrous substance during its passage through the beating devices, stretching the substance so as to detach the elements of the fibers from each other and from the bulk of the fibrous substance, separating the fiber elements by directing liquid jets against the fibrous substance, depriving the separated fiber elements of liquid, and drying said fiber elements.

8. In a process for producing textile

fibers consisting of the separated natural elements of fiber which, in its natural state, consists of long fibers composed of cohering natural elements or cells, deshiving the long fibers, softening the cementitious substance that holds the natural elements together, and then stretching the long fibers to divide them into their elements.

9. In a process for producing textile fibers  
10 consisting of the separated natural elements  
of fiber which, in its natural state, consists of  
long fibers composed of cohering natural ele-  
ments or cells, deshiving the long fibers,  
beating and wetting the long fibers, and then  
15 stretching the long fibers to divide them into  
their elements.

10. In a process for producing textile fibers consisting of the separated natural elements of fiber which, in its natural state, consists of long fibers composed of cohering natural elements or cells, deshiving the long fibers, softening the cementitious substance that holds the natural elements together, stretching the long fibers to divide them into their elements, and washing them to obtain clean fiber-elements properly detached from each other.

11. In a process for producing textile fibers consisting of the separated natural elements of fiber which, in its natural state, consists of long fibers composed of cohering natural elements or cells, deshiving the long fibers, beating and wetting the long fibers, stretching the long fibers to divide them into their elements, and then washing them to obtain clean fiber-elements properly detached from each other.

40 12. In a process for producing textile fibers consisting of the separated natural elements of fiber which, in its natural state, consists of long fibers composed of cohering natural elements or cells, deshiving the long fibers, softening the cementitious substance that holds the natural elements together, 45 stretching the long fibers to divide them into their elements, and then directing liquid jets against the fibers to obtain clean fiber-elements properly detached from each other.

50 13. In a process for producing textile fibers consisting of the separated natural elements of fiber which, in its natural state, consists of long fibers composed of cohering natural elements, deshiving the long fibers, softening the cementitious substance, that holds the natural elements together, stretching the long fibers to divide them into their elements, washing them to obtain clean fiber-elements, and bleaching them.

60 14. In a process for producing textile fibers consisting of the separated natural elements of fiber which, in its natural state, consists of long fibers composed of cohering natural elements, deshiving the long fibers, softening the cementitious substance that holds the natural elements together, stretch-

ing the long fibers to divide them into their elements, washing them to obtain clean fiber-elements, bleaching and sizing them.

15. In a process for producing textile fibers consisting of the separated natural elements of fiber which, in its natural state, consists of long fibers composed of cohering natural elements, deshiving the long fibers, softening the cementitious substance that holds the natural elements together, stretching the long fibers to divide them into their elements, washing them to obtain clean fiber-elements, bleaching, sizing and dyeing them. 70 75

16. In a process for producing textile fibers consisting of the separated natural elements of fiber which, in its natural state, consists of long fibers composed of cohering natural elements, deshiving the long fibers, softening the cementitious substance that holds the natural elements together, stretching the long fibers to divide them into their elements, washing them to obtain clean fiber-elements, and then drying them. 80 85

17. In a process for producing textile fibers consisting of the separated natural elements of fiber which, in its natural state, consists of long fibers composed of cohering natural elements, deshiving the long fibers, softening the cementitious substance that holds the natural elements together, stretching the long fibers to divide them into their elements, washing them to obtain clean fiber elements, bleaching and then drying them. 90  
95

18. In a process for producing textile fibers consisting of the separated natural elements of fiber which, in its natural state, consists of long fibers composed of cohering natural elements, deshiving the long fibers, softening the cementitious substance that holds the natural elements together, stretching the long fibers to divide them into their elements, washing them to obtain clean fiber-elements, bleaching, sizing and then drying them. 100  
105

19. In a process for producing textile fibers consisting of the separated natural elements of fiber which, in its natural state, consists of long fibers composed of cohering natural elements, deshiving the long fibers, softening the cementitious substance that holds the natural elements together, stretching the long fibers to divide them into their elements, washing them to obtain clean fiber-elements, bleaching, sizing, dyeing and then drying them. 110 115 120

20. In a process for producing textile fibres consisting of the separated natural elements of fiber which, in its natural state, consists of long fibers composed of cohering natural elements or cells, deshiving the long fibers, softening the cementitious substance that holds the natural elements together, stretching the long fibers to divide them into their elements, and then directing liquid jets against the fibers to obtain clean fiber- 125  
130

- 6
- elements properly detached from each other, all said steps in the process taking place automatically in a continuous operation.
- 5 21. Apparatus for producing, in a continuous operation, short fibers consisting of the natural elements of fiber which, in its natural state, consists of long fibers composed of cohering natural elements or fiber-cells.
- 10 22. Apparatus for producing, in a continuous operation, short fibers consisting of the natural elements of fiber which, in its natural state, consists of long fibers each composed of cohering natural elements or fiber-cells, said apparatus comprising a softening device for softening the cementitious substance that holds the natural elements of the long fibers together, a stretching device consisting of pairs of fiber-gripping rolls operating successively, the first pair having a lower circumferential speed than the next, and a washing device for cleaning the divided fiber-elements.
- 15 23. Apparatus for producing, in a continuous operation, short fibers consisting of the natural elements of fiber which, in its natural state, consists of long fibers each composed of cohering natural elements or fiber-cells, said apparatus comprising a softening device consisting of cooperating fiber-beaters and water-jets, a stretching device consisting of pairs of fiber-gripping rolls operating successively, the first pair having a lower circumferential speed than the next, and a washing device for cleaning the divided fiber-elements.
- 20 24. Apparatus for producing, in a continuous operation, short fibers consisting of the natural elements of fiber which, in its natural state, consists of long fibers each composed of cohering natural elements or fiber-cells, said apparatus comprising a softening device consisting of cooperating fiber-beaters and water-jets, a stretching device consisting of pairs of fiber-gripping rolls operating successively, the first pair having a lower circumferential speed than the next, and a washing device consisting of strong jets of water directed against the divided individual cells.
- 25 25. Vegetable textile fibers consisting of the separated natural elements of fiber which, in its natural state, consists of long fibers each composed of cohering natural elements or cells.
- 30 26. Vegetable textile fibers consisting of the separated natural elements of fiber which, in its natural state, consists of long fibers composed of cohering natural elements or cells of approximately the length of cotton.
- 35 27. Cottonized fibers produced by treating fibrous substance so as to soften its fibers, stretching the substance to detach the elements of the fibers from each other and separating the fiber elements and washing the fibrous substance by directing liquid jets against it.
- In testimony whereof we affix our signatures.
- BRUNO POSSANNER von EHRENTHAL.  
KARL SCHOLZ.